

Oct. 30, 1962

C. G. BIEBER

3,061,426

CREEP RESISTANT ALLOY

Filed Feb. 1, 1960



CLARENCE G. BIEBER  
INVENTOR.

BY

*C. G. Bieber*  
ATTORNEY

## 1

3,061,426

## CREEP RESISTANT ALLOY

Clarence G. Bieber, West Roselle Park, N.J., assignor to  
The International Nickel Company, Inc., New York,  
N.Y., a corporation of Delaware

Filed Feb. 1, 1960, Ser. No. 6,001

4 Claims. (Cl. 75—171)

The present invention relates to strong heat- and corrosion-resistant alloys and, more particularly, to strong, heat- and corrosion-resistant nickel-chromium-cobalt alloys.

Heretofore, the art has endeavored to provide castable alloys which may be subjected in use to temperatures in excess of about 1700° F. in corrosive atmospheres and which maintain adequate strength and ductility under these conditions. In order to be completely satisfactory, the alloys must not depend upon scarce or expensive elements in order to obtain the required strength at high temperatures. Although attempts were made to overcome the foregoing difficulties and other disadvantages, none, as far as I am aware, was entirely successful when carried into practice commercially on an industrial scale.

It has now been discovered that by the use of a specially coordinated combination of readily obtainable elements, it is possible to produce alloys having substantially enhanced properties when exposed in use to high stresses at elevated temperatures of the order of about 1700° F. and higher.

It is an object of the present invention to provide a novel alloy having substantially enhanced characteristics at elevated temperatures and particularly at temperatures in excess of about 1700° F.

Another object of the invention is to provide a novel heat-resistant article having substantially enhanced characteristics at temperatures in excess of about 1700° F.

The invention also contemplates providing a novel turbine structure having substantially enhanced characteristics at temperatures in excess of about 1700° F.

It is a further object of the invention to provide a novel turbine blade having substantially enhanced characteristics at temperatures in excess of about 1700° F.

Other objects and advantages will become apparent from the following description taken in conjunction with the accompanying drawing in which the FIGURE is a graph relating stress and a parameter commonly known as the Larson-Miller parameter.

Generally speaking, the present invention contemplates novel nickel-chromium-cobalt alloys and articles, structures, etc., made therefrom having substantially enhanced characteristics at elevated temperatures, and, particularly when subjected to temperatures in excess of about 1700° F., comprising about 6% to about 12% chromium, about 5% to about 30% cobalt, about 1% to about 8% molybdenum, about 0.2% to about 2% vanadium, about 4% to about 9% aluminum, about 0.5% to about 6.5% titanium, about 8% to about 12% aluminum plus titanium, about 0.001% to about 0.1% boron, about 0.01% to about 0.25% zirconium, about 0.01% to about 0.5% carbon, with the balance being essentially nickel. The term "balance essentially" is used to include in addition to nickel in the balance of the alloy, small amounts of impurities such as sulfur, phosphorous, etc., and incidental elements such as niobium, tantalum, manganese, silicon, copper, iron, etc., in amounts which do not adversely affect the novel advantageous characteristics of

## 2

the alloy. The novel alloys of the present invention can contain up to about 5% niobium, up to about 2% copper, up to about 1% silicon, up to about 2% manganese, up to about 0.2% calcium, up to about 4% tantalum and up to about 10% iron and more advantageously, up to about 2% iron.

The alloys of the present invention exhibit excellent lives to rupture at elevated temperatures, for example, up to at least about 100 hours life when tested under 10 a load of 35,000 pounds per square inch (p.s.i.) at 1700° F. in combination with a reasonable amount of ductility, for example, at least about 4% elongation under the aforesaid conditions. The alloys can be used in the as-cast condition but can advantageously be treated 15 by heating for about 1/2 to about 4 hours at a temperature of about 2100° F. to about 2200° F. under an inert atmosphere such as helium, argon, etc. The alloys are then cooled rather rapidly to a temperature below about 1700° F. while maintaining them in an inert 20 atmosphere. The alloys and articles made therefrom may be aged in service or may be aged by heating for about 1 to about 20 hours at temperatures of about 1400° F. to about 1700° F. It is characteristic of the 25 alloys of the present invention that they can be readily cast and that they give excellent mold reproduction making them especially suited for use in the precision casting process. The alloys are usually melted from either a calculated charge or from remelt stock under an inert atmosphere (including vacuum) and are cast at temperatures between about 2500° F. and about 3100° F. into molds preheated to about 1000° F. to about 1800° F. If melted at atmospheric pressure a final treatment with calcium silicide prior to casting is advantageous. When produced in this manner, alloys in accordance 30 with the invention may be subjected in use under oxidizing conditions to temperatures up to about 2100° F.

In carrying the invention into practice, it is most advantageous to maintain the composition of the novel alloys within the limited range set forth in Table I.

| Element           | Range, percent |
|-------------------|----------------|
| Chromium          | 8-12           |
| Cobalt            | 10-20          |
| Molybdenum        | 2-5            |
| Vanadium          | 0.25-1.50      |
| Aluminum          | 5-8            |
| Titanium          | 1-6            |
| Aluminum+titanium | 9-11           |
| Carbon            | 0.1-0.3        |
| Boron             | 0.005-0.05     |
| Zirconium         | 0.05-0.1       |
| Nickel            | Balance        |

55 Alloys within the limited range set forth in Table I exhibit lives to rupture in excess of about 100 hours when subjected to a load of 35,000 p.s.i. at 1700° F. and elongations in the range of about 3% to about 20% under the same testing conditions. It is advantageous to maintain a relationship between the vanadium and carbon 60 contents of the alloys as set forth both broadly and in the more advantageous aspects in such fashion that the percentage of vanadium is at least twice the percentage of carbon. Examples of alloy compositions within the scope of the present invention are set forth 65 in Table II together with an outstanding composition selected from the prior art alloys.

Table II

| Alloy No. | Percent Cr | Percent Co | Percent Mo | Percent Al | Percent V | Percent Ti | Percent Cb <sup>1</sup> | Percent C | Percent B | Percent Zr | Percent Ni <sup>2</sup> |
|-----------|------------|------------|------------|------------|-----------|------------|-------------------------|-----------|-----------|------------|-------------------------|
| 1         | 10         | 15         | 3          | 5.5        | 1         | 4.5        | -----                   | 0.18      | 0.02      | 0.05       | Bal.                    |
| 2         | 10         | 20         | 3          | 5.5        | 1         | 4.5        | -----                   | 0.18      | 0.02      | 0.05       | Bal.                    |
| 3         | 10         | 20         | 3          | 5.5        | 1         | 5.0        | -----                   | 0.18      | 0.02      | 0.05       | Bal.                    |
| 4         | 10         | 15         | 3          | 5.5        | 1         | 5.0        | -----                   | 0.18      | 0.02      | 0.05       | Bal.                    |
| 5         | 12         | 15         | 2          | 5.5        | 1         | 4.5        | -----                   | 0.18      | 0.02      | 0.05       | Bal.                    |
| 6         | 10         | 15         | 3          | 5.5        | 1         | 5.5        | -----                   | 0.18      | 0.02      | 0.05       | Bal.                    |
| 7         | 10         | 15         | 3          | 5.7        | 1         | 4.5        | -----                   | 0.18      | 0.02      | 0.05       | Bal.                    |
| 8         | 10         | 15         | 3          | 5.5        | 0.5       | 5.0        | -----                   | 0.18      | 0.02      | 0.05       | Bal.                    |
| 9         | 10         | 15         | 3          | 5.5        | 1         | 4.5        | 1                       | 0.18      | 0.02      | 0.05       | Bal.                    |
| A         | 12         | -----      | 5          | 6          | -----     | 0.6        | 2                       | 0.12      | 0.02      | 0.50       | Bal.                    |

<sup>1</sup> Including small incidental amounts of tantalum.<sup>2</sup> Including small incidental amounts of manganese, silicon, iron, etc.

Alloy No. A is representative of the best commercial alloys of the prior art. Alloys set forth in Table II were produced in various conditions as set forth in Table III and were stress-rupture tested under the conditions set forth in Table IV.

Table III

| Treatment designation | Processing <sup>1</sup> treatment |
|-----------------------|-----------------------------------|
| a                     | A.M. as cast.                     |
| a'                    | V.M. as cast.                     |
| b                     | A.M. 2 hours at 2,150° F.         |
| b'                    | V.M. 2 hours at 2,150° F.         |

<sup>1</sup> A.M.=Melted at atmospheric pressure under argon. V.M.=Melted under vacuum.

Table IV

| Test designation | Temperature, ° F. | Stress, p.s.i. |
|------------------|-------------------|----------------|
| S                | 1,600             | 60,000         |
| T                | 1,700             | 40,000         |
| U                | 1,700             | 35,000         |
| V                | 1,800             | 25,000         |
| W                | 1,800             | 20,000         |
| X                | 1,850             | 20,000         |
| Y                | 1,900             | 15,000         |
| Z                | 1,900             | 16,000         |

The results of life-to-rupture tests conducted on alloys set forth in Table II which were heat treated as set forth in Table III and tested under the conditions set forth in Table IV, are presented in Table V. Standard specimens having gage sections 0.250 inch in diameter and 1.0 inch in length were used for these test purposes.

Table V

| Alloy No. | Processing treatment | Test condition | Time to fracture, hours | Elongation, percent |
|-----------|----------------------|----------------|-------------------------|---------------------|
| 1         | a'                   | U              | 146.9                   | 7                   |
| 2         | a'                   | U              | 122.4                   | 8.0                 |
| 3         | a'                   | U              | 128.3                   | 7                   |
| 4         | a                    | U              | 119.8                   | 7.4                 |
| 4         | b                    | V              | 122.3                   | 10.6                |
| 4         | b                    | X              | 95.1                    | 11.5                |
| 4         | b                    | Y              | 131.0                   | 10.6                |
| 5         | b'                   | X              | 77.9                    | 4.8                 |
| 5         | b'                   | W              | 413.0                   | 9.8                 |
| 6         | b'                   | U              | 183.2                   | 4.4                 |
| 6         | b'                   | U              | 153.0                   | 4.4                 |
| 6         | b'                   | T              | 92.5                    | 2.2                 |
| 7         | b'                   | X              | 99.4                    | 9.7                 |
| 7         | b'                   | S              | 79.4                    | 3.5                 |
| 8         | b'                   | U              | 192.6                   | 4.4                 |
| 8         | b'                   | Z              | 82.4                    | 4.0                 |
| A         | a                    | U              | 24                      | 6                   |

It is characteristic of the alloys of the present invention that they exhibit, in addition to high strength at elevated temperatures, good resistance to thermal shock. When

tested by repeatedly subjecting airfoil turbine blade sections to an intermittent heating and cooling cycle comprising heating in a flame for one minute to 1800° F. and then cooling in air for one minute, the alloys of the present invention withstand many thousand cycles without failure. For example, one alloy in accordance with the present invention withstood 5850 cycles prior to failure as indicated by the formation of the first crack 0.125 inch in length. Under same conditions prior art alloys in commercial use fail in one to two thousand cycles.

Referring now to the drawing, it is to be observed that the stress rupture characteristics of an alloy in accordance with the present invention containing about 10% chromium, 15% cobalt, 3% molybdenum, 5.5% aluminum, 5.0% titanium, 0.18% carbon, 0.02% boron, 0.05% zirconium, 1% vanadium and the balance essentially nickel, which was heat treated at 2150° F. for two hours and then air cooled, can be illustrated in the manner suggested by Larson and Miller (see Transactions of the A.S.M.E., 1952, volume 74, pages 765-771). It is to be noted that the figure shows a master curve for the aforementioned alloy obtained by plotting "stress $\times$ 1000 p.s.i." against "P" (parameter). Parameter "P" is obtained from experimental data by the use of the following formula

$$P = T(C + \log t) \times 10^{-3}$$

wherein

$P$ =parameter,

$T$ =absolute temperature in ° Rankine,

$\log t$ =common logarithm of the time to rupture in hours; and

$C$ =a constant having a value of 25.

Through the use of this master curve together with a knowledge of a desired stress temperature combination one is able to calculate either graphically or mathematically the life to rupture exhibited under selected conditions within the range of experience.

In general, alloys produced in accordance with the present invention have 100 hour rupture strengths at various temperatures of the order of those shown in Table VI.

Table VI

| Temperature, ° F. | Rupture strengths, p.s.i. |
|-------------------|---------------------------|
| 1500              | 72,000-78,000             |
| 1600              | 54,000-60,000             |
| 1700              | 36,000-42,000             |
| 1800              | 24,000-28,000             |
| 1900              | 13,000-18,000             |

In addition to excellent rupture strengths the alloys of the present invention also exhibit excellent short-time tensile characteristics at temperatures ranging from room temperature up to and including 1800° F. Short-time tensile characteristics measured on the short-time high temperature test scale for alloy No. 1 as set forth in Table II are presented in Table VII.

5  
Table VII

| Test temperature | 0.2% yield strength, p.s.i. | Strength, p.s.i. | Elongation, percent | Reduction in area, percent |
|------------------|-----------------------------|------------------|---------------------|----------------------------|
| Room temp.       | 115,000                     | 135,750          | 10.8                | 18.1                       |
| Do.              |                             | 135,000          | 8.0                 |                            |
| 1,200° F.        | 118,000                     | 145,250          | 9.0                 | 10.9                       |
| 1,200° F.        | 106,000                     | 123,750          | 7.0                 | 11.6                       |
| 1,500° F.        | 127,250                     | 135,000          | 3.0                 | 4.1                        |
| 1,500° F.        | 128,250                     | 136,000          | 7.0                 | 3.3                        |
| 1,600° F.        | 97,300                      | 114,000          | 5.0                 | 5.5                        |
| 1,600° F.        | 101,000                     | 121,750          | 4.4                 | 3.1                        |
| 1,800° F.        | 56,750                      | 76,750           | 4.4                 | 8.7                        |
| 1,800° F.        | 60,000                      | 76,250           | 4.4                 | 8.4                        |

Additional alloys in accordance with the present invention are set forth in Table VIII.

Table VIII

| Alloy No. | Percent Cr | Percent Co | Percent Mo | Percent Al | Percent Ti | Percent V | Percent C | Percent B | Percent Zr | Percent Ni <sup>1</sup> |
|-----------|------------|------------|------------|------------|------------|-----------|-----------|-----------|------------|-------------------------|
| 10.       | 9.37       | 8.41       | 2.99       | 5.95       | 5.06       | 0.97      | 0.14      | 0.014     | 0.04       | Bal.                    |
| 11.       | 9.78       | 14.54      | 3.00       | 6.10       | 5.36       | 1.01      | 0.15      | 0.018     | 0.05       | Bal.                    |
| 12.       | 10.03      | 8.8        | 3.13       | 6.00       | 5.5        | 0.97      | 0.15      | 0.023     | 0.05       | Bal.                    |
| 13.       | 9.92       | 14.74      | 3.03       | 5.96       | 3.33       | 0.94      | 0.19      | 0.017     | 0.04       | Bal.                    |

<sup>1</sup> Including small incidental amounts of silicon, manganese, iron, etc.

Each of the aforementioned alloys Nos. 10 to 13 which were vacuum melted and heat treated at 2150° F. for 2 hours and then cooled, exhibited a 100 hour rupture life under the specific stress-temperature conditions as set forth in Table IX.

Table IX

| Alloy No. | Temperature, ° F. | Stress for 100 hour rupture life, p.s.i. |
|-----------|-------------------|------------------------------------------|
| 10.       | 1,900             | 14,000                                   |
| 11.       | 1,900             | 13,000                                   |
| 12.       | 2,000             | 9,000                                    |
| 13.       | 1,900             | 16,000                                   |

The present invention is particularly applicable to the production of alloys employed in gas turbine structures such as rotor blades, stator blades, nozzle guide vanes, rotors, etc. The novel alloys of the present invention may also be used as extrusion dies, valves, valve seats, etc.

Although the present invention has been described in conjunction with preferred embodiments, it is to be understood that modifications and variations may be restored to without departing from the spirit and scope of the invention, as those skilled in the art will readily understand. Such modifications and variations are considered to be within the purview and scope of the invention and appended claims.

I claim:

1. An alloy for use as castings and characterized by a prolonged life to rupture when exposed at elevated temperatures to the combined effects of applied stress and an oxidizing atmosphere containing about 6% to about 12% chromium, about 5% to about 30% cobalt, about 1% to about 8% molybdenum, about 8% to about 12% aluminum plus titanium, about 4% to about 9% aluminum, about 0.5% to about 6.5% titanium, about 0.2% to about 2% vanadium, about 0.001% to about 0.1% boron, about

0.01% to about 0.25% zirconium, about 0.01% to about 0.5% carbon with the balance being essentially nickel.

2. An alloy for use as castings and characterized by having a life to rupture of at least about 100 hours when exposed at a temperature of 1700° F. to a load of 35,000 pounds per square inch containing about 8% to about 12% chromium, about 10% to about 20% cobalt, about 2% to about 5% molybdenum, about 9% to about 11% aluminum plus titanium, about 5% to about 8% aluminum, about 1% to about 6% titanium, about 0.25% to about 1.50% vanadium, about 0.005% to about 0.05% boron, about 0.05% to about 0.1% zirconium, about 0.1% to about 0.3% carbon with the balance being essentially nickel.

15

3. An alloy for use as castings and characterized by having a life to rupture of at least about 100 hours when exposed at a temperature of 1700° F. to a load of 35,000 pounds per square inch containing about 8% to about 12% chromium, about 10% to about 20% cobalt, about 2% to about 5% molybdenum, about 9% to about 11% aluminum plus titanium, about 5% to about 8% aluminum, about 1% to about 6% titanium, about 0.25% to about 1.50% vanadium, about 0.005% to about 0.05% boron, about 0.05% to about 0.1% zirconium, about 0.1% to about 0.3% carbon, with the balance being essentially nickel, the carbon and vanadium contents of said alloy being so related that the vanadium percentage is at least twice the carbon percentage.

4. An alloy for use as castings and characterized by a prolonged life to rupture when exposed at elevated temperatures to the combined effects of applied stress and an oxidizing atmosphere containing about 6% to about 12% chromium, about 5% to about 30% cobalt, about 1% to about 8% molybdenum, about 8% to about 12% aluminum plus titanium, about 4% to about 9% aluminum, about 0.5% to about 6.5% titanium, about 0.2% to about 2% vanadium, about 0.001% to about 0.1% boron, about

45

50

55

0.01% to about 0.25% zirconium, about 0.01% to about 0.5% carbon, with the balance being essentially nickel, the carbon and vanadium contents of said alloy being so related that the vanadium percentage is at least twice the carbon percentage.

#### References Cited in the file of this patent

#### UNITED STATES PATENTS

60 2,912,323 Bieber et al. ----- Nov. 10, 1959  
2,920,956 Nisbet et al. ----- Jan. 12, 1960

#### OTHER REFERENCES

Journal of Metals, vol. 5, September 1953 (Nisbet et al.)  
65 (pages 1149-1165 relied upon).

UNITED STATES PATENT OFFICE  
CERTIFICATE OF CORRECTION

Patent No. 3,361,426

October 30, 1962

Clarence G. Bieber

It is hereby certified that error appears in the above numbered patent requiring correction and that the said Letters Patent should read as corrected below.

Columns 3 and 4, Table II, eleventh column, line 10 thereof, for "0.50" read -- 0.05 --; columns 5 and 6, Table VIII, tenth column, line 3 thereof, for "0.05" read -- 0.04 --.

Signed and sealed this 21st day of May 1963.

(SEAL)

Attest:

RNEST W. SWIDER  
Attesting Officer

DAVID L. LADD  
Commissioner of Patents